

## UNITED STATES PATENT OFFICE

2,138,771

## LUBRICATING OIL

Ernest F. Pevere, Beacon, N. Y., assignor to The Texas Company, New York, N. Y., a corporation of Delaware

No Drawing. Application June 23, 1934.  
Serial No. 732,092

7 Claims. (Cl. 87—9)

This invention relates to the manufacture of lubricating oil characterized by a low pour test and/or an increased viscosity index.

The invention contemplates the preparation of mineral lubricating oil having a reduced pour test and other desired qualities from lubricating oil stock, such as those derived from mixed base and paraffin base crudes and the like, by the addition to the lubricating oil of a pour point depressant material or wax crystal inhibitor. The invention particularly contemplates the addition to a lubricating oil of a small proportion of a higher fatty acid ester of a higher aliphatic alcohol having 6 or more carbon atoms to the molecule, such as mannnitan tetrastearate.

The invention also contemplates the preparation of mineral lubricating oil having an increased viscosity index from naphthene base crudes as well as mixed base and paraffin base crudes, by the addition to the lubricating oil of a minor proportion of the same fatty acid esters of higher aliphatic alcohols.

Lubricating oil stocks derived from paraffin and mixed base crudes contain appreciable amounts of wax and, therefore, have a relatively high pour test unless a substantial amount of this wax is removed. The removal of this wax is usually accomplished by cold settling, filtration or centrifuging. However, lubricating oil stocks, after dewaxing by these processes, may still retain some wax, and may have a pour test above 15° F. and up to about 40° F. The removal of further quantities of wax from these stocks in order to further reduce the pour test necessitates expensive further processing.

On the other hand, the presence of a certain amount of wax in a lubricating oil may be beneficial from the standpoint of providing a comparatively flat temperature-viscosity curve. That is, there is a relatively small change in the viscosity of the oil between temperatures of say 100° F. and 210° F. Consequently, it is of advantage to add to the oil a material which will have the effect of reducing the pour test or cold test to the desired extent without the necessity of entirely removing the remaining wax.

I have discovered that a higher fatty acid ester of a higher aliphatic alcohol having 6 or more carbon atoms to the molecule constitutes an effective material for addition to a partially dewaxed mineral lubricating oil of this character to lower the pour point thereof. Fatty acid esters, particularly from the saturated higher fatty acids including stearic and palmitic acids, with the higher aliphatic monohydric alcohols, including

hexyl, heptyl, octyl and cetyl, and the hexahydric alcohols such as mannitol and sorbitol, are representative of this class of compounds.

In the production of high grade lubricating oils, it is well known that a relatively small change in the viscosity of the oil between temperatures of say 100° F. and 210° F., is desirable. In other words, it is advantageous for the oil to have a relatively flat viscosity-temperature curve, which means that the oil has a high viscosity index as defined by Dean and Davis in their article in Chemical and Metallurgical Engineering, vol. 36, page 618. Improvement in lubricating oils has heretofore been accomplished by refining, as by the use of selective solvents which are effective in extracting or separating naphthenic constituents from paraffinic constituents, thereby producing a resulting raffinate of increased viscosity index. This procedure involves expensive processing, and results in a reduced yield of finished oil.

The addition of an ester selected from the class of compounds enumerated above in controlled proportions to a naphthene base or paraffin base lubricating oil is also found to materially increase the viscosity index thereof, without objectionably affecting other desirable properties. When the esters are added to improve the viscosity index of a lubricating oil, a proportion of about 5-15% by weight is generally employed. On the other hand, where reduction in pour point of a partially dewaxed paraffin base lubricating oil is desired, a smaller proportion of such an ester may be employed with resulting economy. For example, as little as  $\frac{1}{4}$  of 1% by weight of the ester will effect substantial reduction in pour point, and a proportion range of about  $\frac{1}{4}\%$  to  $\frac{1}{2}\%$  is generally employed.

By way of example, mannnitan tetrastearate was prepared by heating 1 mol of mannitol and 4 mols of commercial stearic acid together under sub-atmospheric pressure at temperatures of 200°-250° C. The reaction product was then purified by crystallization from ethyl alcohol, thereby removing free fatty acid. The purified product was then added to a partially dewaxed paraffin base lubricating oil having a pour point of +20° F. with the following results:

| 100 cc. paraffin base lubricating oil plus— | Pour point | 50 |
|---------------------------------------------|------------|----|
| °F.                                         |            |    |
| 0.125 g. mannnitan tetrastearate.....       | +10        |    |
| 0.25 g. mannnitan tetrastearate.....        | 0          |    |
| 0.50 g. mannnitan tetrastearate.....        | -5         |    |

A portion of the mannitan tetrastearate prepared as outlined above was added to a naphthene base lubricating oil in the proportion of 5% by weight with the following results:

5

|                            | Naphthene<br>base lube<br>oil | 95% naphthene<br>base lube oil,<br>5% mannitan<br>tetrastearate |
|----------------------------|-------------------------------|-----------------------------------------------------------------|
| 10 Saybolt vis. at 100° F. | 530                           | 499                                                             |
| 10 Saybolt vis. at 210° F. | 52                            | 54                                                              |
| 10 Viscosity index         | 2                             | 29                                                              |

As a further example, cetyl palmitate was prepared by heating cetyl alcohol and palmityl chloride together on a water bath in the proportions of 20 g. of cetyl alcohol to 22 g. of palmityl chloride, until the evolution of HCl ceased. The product so obtained was purified by repeated crystallization from ethyl alcohol, and was dried over calcium chloride. The cetyl palmitate was added to a naphthene base oil in the proportion of 5% by weight with the following results:

15

|                            | Naphthene<br>base lube<br>oil | 95% naphthene<br>base lube oil,<br>5% cetyl pal-<br>mitate |
|----------------------------|-------------------------------|------------------------------------------------------------|
| 20 Saybolt vis. at 100° F. | 530                           | 400                                                        |
| 20 Saybolt vis. at 210° F. | 52                            | 51                                                         |
| 20 Viscosity index         | 2                             | 32.5                                                       |

Where the expression "paraffin base lubricating oil" is used in the accompanying description and claims, it is to be understood that this refers to an oil of the mixed base or Mid-Continent type as well as an oil of the paraffin base or Pennsylvania type, unless the contrary appears from the text.

Obviously many modifications and variations of the invention, as hereinbefore set forth, may be made without departing from the spirit and scope thereof, and therefore only such limitations should be imposed as are indicated in the 5 appended claims.

I claim:

1. A lubricating oil comprising a mixture of a petroleum lubricating oil with a minor proportion of a higher saturated fatty acid ester of 10 mannitol.

2. A lubricating oil comprising a mixture of a petroleum lubricating oil with a minor proportion of mannitan tetrastearate.

3. A lubricating oil having a pour point of approximately 5° F. or below comprising a mixture of a partially dewaxed paraffin base lubricating oil normally having a pour point above 15° F. with mannitan tetrastearate in the proportion of about 1/4% to 1 1/2% by weight.

4. A lubricating oil having a relatively higher viscosity index comprising a petroleum lubricating oil having a relatively lower viscosity index admixed with about 5-15% by weight of a higher saturated fatty acid ester of mannitol.

5. A lubricating oil having a relatively higher viscosity index comprising a petroleum lubricating oil having a relatively lower viscosity index admixed with about 5-15% by weight of mannitan tetrastearate.

6. A lubricating oil comprising a mixture of a petroleum lubricating oil with a minor proportion of a higher fatty acid ester of a hexahydric alcohol selected from the group consisting of mannitol and sorbitol.

7. A lubricating oil as defined in claim 6, in which the ester is substantially devoid of free fatty acid.

ERNEST F. PEVERE.